

March 5, 1957

H. H. E. SCHARF ET AL

2,783,967

CERAMIC MACHINE PARTS

Filed Dec. 24, 1952

FIG-1



FIG-2



INVENTORS  
HERBERT SCHARF,  
RUDOLF SCHMUCKER &  
WALTER RICHTER

BY *Marshall, Biobel, French & Buzz*  
ATTORNEYS

# United States Patent Office

2,783,967

Patented Mar. 5, 1957

1

2,783,967

## CERAMIC MACHINE PARTS

Herbert H. E. Scharf, Rudolf W. F. Schmucker, and Walter Richter, Augsburg, Germany, assignors to Maschinenfabrik Augsburg-Nürnberg A. G., Augsburg, Germany, a corporation of Germany

Application December 24, 1952, Serial No. 327,716

Claims priority, application Germany January 3, 1952

3 Claims. (Cl. 253—77)

This invention relates to ceramic machine parts, and more particularly to the manufacture of ceramic turbine blades for mounting in a metal rotor rim.

Ceramic materials have been found appropriate for turbine blades and similar parts of high temperature gas turbines because of the thermal properties of ceramics. Many ceramic materials, however, exhibit low mechanical strength despite their desirable thermal properties. Accordingly, special measures must be taken to increase the mechanical strength or stability of certain ceramic materials if it is desired to use them, for example, in high temperature gas turbine blades.

It has been found that coating the ceramic material with a glaze substantially increases the tensile strength of the ceramic. At the same time, however, such a glaze notably increases the weight of the ceramic material. Such increased weight, particularly on the leaf or vane portion of a turbine blade, may not be desirable since it correspondingly increases the centrifugal force to which the blade is subjected as well as increasing the brittleness of the ceramic in the part of the blade which is most subjected to oscillation and vibration in operation of the turbine.

It is accordingly a principal object of this invention to produce a turbine blade with a strength-increasing glaze applied only to highly strained portions of the blade.

A further object of the invention is to apply a glaze the linear thermal expansion coefficient of which is smaller than that of the blade material for increasing mechanical stability.

Another object of this invention is to provide a ceramic turbine blade with a stability-increasing glaze applied to but portions thereof and with the transition points between unglazed and glazed portions of the blade graduated.

A further object of this invention is to provide a ceramic turbine blade having on the root portions thereof engaged by a metal turbine rotor a layer of strength-increasing glaze and an additional layer of machinable material to provide for close tolerance fitting of said blades without disturbing surface equilibrium of said glaze or said blade.

Still another object of this invention is to provide a ceramic turbine blade with the root portions thereof carrying a strength-increasing glaze the amount of which is graduated at the transition point between glazed and unglazed portions of the blade.

Still another object of this invention is to provide a ceramic turbine blade having on selected highly strained portions thereof, such as the root portion seating surfaces and the thin trailing edge of the vane, a strength-increasing glaze with a lower coefficient of thermal expansion than the ceramic material from which the blade is formed.

Other objects and advantages will be apparent from the following description, and the appended claims.

In the drawing:

2

Fig. 1 shows a front view of a blade embodying this invention; and

Fig. 2 shows a side view of a blade embodying this invention.

Referring to the drawing, the turbine blade is formed of fired ceramic material and has a root portion 10 for engagement in the rim of a metal turbine rotor and a vane portion 11. As indicated by shading on the drawing, the root portion 10 is covered with a glaze. The vane portion 11 is unglazed. At the transition area 12 between the glazed root and the unglazed vane the thickness of the applied glaze decreases either gradually or stepwise. Preferably this graduated thickness decreases in at least two steps between the glazed root 10 and the unglazed vane 11. As a result of the internal conditions achieved in the firing of the ceramic material as well as the increased stability imparted to the glazed portion of the blade, the transition between glazed and unglazed portions might produce a point of weakness unless this transition were graduated.

The vane portion 11 is unglazed to reduce the weight thereof subjected to centrifugal force as well as to avoid excessive embrittlement of the ceramic material of the vane portion 11 which is primarily subjected to oscillation and vibrational forces in operation of the turbine. Since, however, the trailing edge 13 of the vane portion may be quite thin, a thin strip of glaze is applied to this thin trailing edge to increase the mechanical strength thereof in use.

During the firing of the blade the ceramic material acquires certain internal equilibrium conditions which are disruptable by such operations as machining the surface of the fired blade. Such machining operations are, however, frequently desirable on the blade root in order to achieve close tolerance fit of the blade in the metal turbine rotor. Accordingly, a further machinable layer 14 of ceramic material is applied over the seating surfaces of the blade root as a machining allowance in order that necessary machining of the blade root may take place without disruption of the internal strength equilibria of the ceramic blade nor the surface of the strength increasing glaze. Also the glaze provides an insulating layer to protect the fired ceramic from effects of machining the layer 14.

The glaze is selected according to the ceramic material so that the coefficient of thermal expansion of the glaze will be less than that of the ceramic material thereby considerably increasing the strength of the ceramic at high temperature conditions. The glaze is preferably formed on the glazed portion of the ceramic blade during the firing of the blade. By way of example, with a turbine blade formed primarily of the steatite-like materials a satisfactory glaze composition according to this invention comprises by way of example a glaze of the formula of Seger:



Additionally a nonamorphous "firing skin" or a "development glaze" can be obtained on highly stressed portions of the ceramic article by placing on the article, for example, an alkali earth or alkali compound which melts at high temperatures and coats the surface of the ceramic blade with a uniform thin layer. Satisfactory results have been obtained by forming such a firing skin, development glaze and the glaze according to this invention on selected portions of the ceramic blade during the final firing thereof to achieve optimum internal equilibrium conditions.

Thus it will be seen that this invention provides a turbine blade in which selected highly strained portions are

strengthened by the addition of a special glaze material, but with other portions of the blade free of glaze and accordingly unencumbered by either the added weight or added brittleness which a glaze provides. Also, particularly on the machined root portions of the blade, the internal equilibria of the ceramic material are insulated by the glaze by disruption during machining operations, and points of possible weakness at the transition area between glazed and unglazed portions are avoided by stepwise graduation of glaze thickness.

While the method and product herein described constitute preferred embodiments of the invention, it is to be understood that the invention is not limited to this precise method and product, and that changes may be made therein without departing from the scope of the invention which is defined in the appended claims.

What is claimed is:

1. A turbine blade of fired ceramic material having a vane portion and a root portion adapted for mounting in a metal turbine rotor comprising a surface layer of glaze on said root portion only, said vane portion being substantially free of glaze, and a second surface layer of glaze of less thickness than said first layer between said root portion and said vane portion effecting gradual diminution of glaze thickness, the coefficient of thermal expansion of said glaze being less than that of said ceramic material.

10

2. A ceramic turbine blade according to claim 1 having an additional layer of glaze in the form of a thin strip along the trailing edge of said vane portion.

3. A ceramic turbine blade according to claim 1 in which said decrease of glazed layer thickness from said root portion toward said vane portion occurs in at least two stages.

References Cited in the file of this patent

UNITED STATES PATENTS

|           |               |               |
|-----------|---------------|---------------|
| 1,081,542 | Malm          | Dec. 16, 1913 |
| 2,157,100 | Rowland       | May 9, 1939   |
| 2,320,099 | Ramsay et al. | May 25, 1943  |
| 2,431,660 | Gaudenzi      | Nov. 25, 1947 |
| 2,581,252 | Goetzl et al. | Jan. 1, 1952  |
| 2,683,018 | Schorner      | July 6, 1954  |

FOREIGN PATENTS

|         |               |               |
|---------|---------------|---------------|
| 195,050 | Great Britain | July 19, 1923 |
| 664,986 | Great Britain | Jan. 16, 1952 |
| 821,735 | Germany       | Nov. 19, 1951 |
| 892,785 | France        | Jan. 13, 1944 |

OTHER REFERENCES

Ser. No. 385,334, Schutte (A. P. C.), published May 25, 1943.